

## UNITED STATES PATENT OFFICE

MARCEL HIPPOLYTE HUE, OF BOIS-GUILLAUME, FRANCE

## PROCESS FOR MANUFACTURING AGGLOMERATED PRODUCTS

No Drawing. Application filed April 29, 1929, Serial No. 359,167, and in France March 18, 1929.

The present invention relates to a process for the manufacture of agglomerated products from the dust or waste of anthracite or other mineral fuels. The said powder or waste, after a preliminary drying in retort furnaces heated to 1200° C., is ground to a fine powder, which is then loaded into mixing and grinding apparatus together with a suitable binding substance, which according to the invention comprises petroleum pitch, heavy petroleum oil, such as mazout, and a vegetable oil. The mass thus mixed is placed in presses in which the agglomerated products are given the required shape, in the known manner.

The said agglomerated products are then placed in ovens heated to a temperature of 300-400° C. in which they are converted into coke. The duration of the treatment in the ovens is usually 1½ hours. It may vary according to the nature of the fuel.

The said binding substance, which consists of petroleum pitch, heavy petroleum oil and vegetable oil, constitutes the essential feature of the invention. In practice, this material consists of the following mixture:

|                                        | Per cent |
|----------------------------------------|----------|
| Petroleum pitch                        | 65       |
| 30 Mazout or other heavy petroleum oil | 24       |
| Cotton seed oil                        | 6        |
| Water                                  | 5        |

Obviously, these proportions are given solely by way of example, instead of the cotton seed oil, any other vegetable oil can be used.

The said substances are mixed at a temperature of about 60° C. and the petroleum pitch and the mazout are first mixed together, then adding the vegetable oil and the water.

40 The binding substance thus prepared is added to anthracite dust or waste, the proportion being 5 to 25 per cent for the binding substance and 95 to 75 per cent of the 45 anthracite dust or waste.

I claim:

A process for the manufacture of agglomerated products from coal dust, comprising the steps of mixing the coal dust with an agglomerating material composed of 65% petroleum pitch, 24% mazout, and 6% non-oxidizing vegetable oil; then agglomerating the mixture; and finally coking the agglomerate thus obtained.

In testimony whereof I affix my signature. 55  
MARCEL HIPPOLYTE HUE.

50

60

65

66

65

70

75

80

85

85